# EUROPEAN PATENT SPECIFICATION

(11) **EP 0 195 898 B1**
(45) Date of publication and mention of the grant of the patent: **02.11.1988**
(21) Application number: 86101289.6
(22) Date of filing: 31.01.1986
(51) Int. Cl.: C09K 9/02, C09B 67/18, G03C 1/733, C09B 19/00

(54) **A method of increasing the light fatigue resistance of a photochromic composition and photochromic composition**
Verfahren zur Verbesserung der Lichtermüdungsbeständigkeit einer photochromen Zusammensetzung und photochrome Zusammensetzung
Procédé pour améliorer la résistance d'une composition photochromique à la fatigue à la lumière et composition photochromique

(30) Priority: 31.01.1985 US 696452
(43) Date of publication of application: 01.10.1986
(73) Proprietor: AMERICAN OPTICAL CORPORATION, Southbridge, MA 01550 (US)
(72) Inventor: Chu, Nori Y. C., Shrewsbury MA 01545 (US)
(74) Representative: Diehl, Hermann O. Th., Dr.

(56) References cited:
- DD-A- 156 372
- GB-A- 2 117 390
- MODERN PLASTICS ENCYCLOPEDIA, 1983-1984, 5, Pristol, LI, S.S. "Ultraviolet Stabilizers", pp. 174-177

## Description

The invention relates to a method of increasing the light fatigue resistance of a photochromic composition and a photochromic composition. This invention relates more particularly to an organic photochromic composition comprising spiro lindoline-2,3'-[3LH]-napht[2,1-N[lA]oxazine] (S.O.) dye and unconventional ultraviolet (UV) stabilizers.

Compounds which undergo reversible photo-induced color changes are termed photochromic compounds. When subjected to ultraviolet light or visible irradiation, these photochromic compounds change their transmission. They subsequently revert to their original color state when they are subjected to a different wavelength of radiation or when the initial light source is removed.

Although the organic photochromic materials have been known for over 50 years, they have not had widespread industrial or commercial use. This is primarily due to the irreversible decomposition phenomenon, generally known as light fatigue. Repeated exposure to light causes the photochromic materials to lose their photochromism.

It is thought that light or heat or both light and heat are responsible for the photodecomposition of organic photochromic compounds. Thus, many people have tried to increase the light fatigue resistance of the compounds by adding numerous conventional antioxidants or ultraviolet light absorbers. For example, U.S. Patent No. 3 212 898 teaches the use of conventional UV absorbers such as benzophenone and benzotriazole to increase the photochromic life of photochromic benzospiropyran compounds. Similarly, U.S. Patent No. 3 666 352 teaches the use of conventional UV light absorbers in photochromic mercury thiocarbazonate lenses, transparent to radiation of wavelengths greater than 420 nm and opaque to radiation of wavelengths less than 420 nm in order to substantially increase the durability of the lenses against photochemical degradation.

One class of organic photochromic compounds, spiro[indoline-2,3'-[3N-naphth[2,1-bl[1,4]oxazine] dyes (S.O. dyes) are known to have good light fatigue resistance. In general, the light fatigue resistance of the spirooxazine compounds is about 100 times better than the closely related spiropyrans. This class of photochromic compounds has been disclosed in U.S. Patent Nos. 3 562 172; 3 578 602; 4 215 010; 4 342 668; and 4440672.

The precise mechanism for photodecomposition of S.O. dyes is not yet fully understood. Although some circumstantial evidence indicates that oxygen is involved in the photodecomposition process, the traditional antioxidants (aryl amines and hindered phenols) do not improve the light fatigue resistance of S.O. dyes. The conventional UV stabilizers, substituted benzophenones and benzotriazoles, cause a small improvement in the light fatigue resistance of S.O. dyes, but they cannot be used effectively since they create a screening effect by absorbing UV radiation strongly in the region where the S.O. dyes absorb UV radiation. By competing with the S.O. dyes to absorb UV light, these conventional stabilizers substantially decrease the effective light intensity for S.O. dye activation. Furthermore, some of the conventional UV stabilizers are detrimental to S.O. dyes under certain conditions.

In addition, the presence of acids has a deleterious effect on S.O. compounds. Acids may be in the plastic host material from which the photochromic article is made, such as PVC or cellulosics. The acids are usually generated either thermally during the forming process, or photochemically during use of the photochromic article. The S.O. dye solution becomes a pinkish to reddish color in the presence of even a minute amount of acid, and the solution ceases to show a photochromic effect. The pinkish to reddish color is likely due to the formation of a complex between the S.O. compound and acid. A base must be used to neutralize the acid and to restore the original colorless or light blue color.

U.S. Patent No. 4 440 672 discloses the use of organonickel complex stabilizers to improve the light fatigue resistance of the photochromic compounds. However, these organonickel complexes do not have the ability to neutralize acids which may be present.

It is therefore an object of this invention to provide a method of increasing the light fatigue resistance of photochromic compositions. This object is solved by the method according to claim 1. Further advantageous features are evident from the subclaims.

It is a further object of this invention to provide a photochromic composition resistant to fatigue. This object is solved by the photochromic composition according to claim 11. Further advantageous features of this composition are evident from the subclaims.

The problems of the prior art are overcome by the discovery that a group of unconventional UV stabilizers will improve the light-fatigue resistance of S.O. dyes, while not affecting their photocolorability. These unconventional UV stabilizers belong to the class of hindered amine light stabilizers (HALS) and excited state quenchers. Hindered amine light stabilizers offer an advantage over organometallic complex stabilizers in their ability to neutralize acid, and to thus improve the light-fatigue resistance and preserve the original color of the S.O. dyes. It is preferable to use the hindered amine light stabilizers together with excited state quenchers in the organic photochromic compound of the invention; this combination has a synergetic effect in improving the light fatigue resistance of the S.O. compounds.

These UV stabilizers will not hinder the photocolorability of S.O. dyes, since they have a minimal absorption in the UV region where S.O. dyes absorb. The S.O. dye and UV stabilizers may be incorporated within optically clear plastics to make a photochromic element suitable for a photochromic sunglass lens, ski goggle, or other plastics to render them photochromic.

Accordingly, the present invention improves the light fatigue resistance of an organic photochromic composition containing S.O. dye.

The present invention further improves the light fatigue resistance of these photochromic compositions without hindering their photocolorability.

Besides this, the present invention allows to use such improved photochromic compositions to fabricate photochromic articles such as sunglasses, ophtalmic lenses, ski goggles, window coatings, toys, fabrics, and the like.

Other objects and further scope of applicability of the present invention will become apparent from the detailed description to follow.

In the following, a preferred embodiment of the invention will be described.

The organic photochromic composition of the present invention comprises: a) spiro [indoline-2,3'-[3H]-naphth[2,1-b][1,4]oxazine] dye (spirooxazine dye), having the structural formula wherein one of R₁, R₂ and R₃ is hydrogen, halogen, lower alkyl, or lower alkoxy and the others are hydrogen; R₄ and R₅ are hydrogen lower alkyl, lower alkoxy, halogen, or trifluoromethyl; and R₆ is lower alkyl; and, b) an unconventional UV stabilizer or stabilizers. As used throughout the specification and claims, "lower" means up to 12 carbon atoms (n = 1 - 12) in the free alkyl or alkoxy radical group, wherein the alkyl free radical group has the structural formula of CₙH₂ₙ₊₁, and the alkoxy free radical group has the structural formula of CₙH₂ₙ₊₁O. The UV stabilizer comprises a hindered amine light stabilizer (HALS). The preferred hindered amine light stabilizers comprise derivatives of tetramethyl piperidine. Most preferably, the UV stabilizer comprises a combination of a hindered amine light stabilizer and an excited state quencher. Preferably, the excited state quencher comprises an organonickel complex light stabilizer. For a description of hindered amine light stabilizers and excited state quenchers, see the following four articles in Modern Plastics Encyclopedia, which are herein incorporated by reference: 1) Shute, Raymond, "Antioxidants," pp. 102-103 (1983-1984); 2) Li, S.S., "Ultraviolet Stabilizers," pp. 174-177 (1983-1984); 3) Patel, A., "Antioxidants," pp. 106-107 (1984-1985); and 4) Stretanski, J.A., "Ultraviolet Stabilizers," pp. 179-180 (1984-1985).

Between 0.1 and about 15 % by weight of the S.O. dye and between 0.01 and about 5 % by weight of the HALS stabilizer or combined UV stabilizers, depending on their solubility, can be incorporated into a plastic article having enhanced light fatigue resistance. The S.O. dye and UV stabilizers may be mixed in a solution with an optically clear polymer which is thereafter cast as a film, sheet, lens, or toy, or a polymer which is injection molded or otherwise shaped into a film or lens; or a prepolymerized film or lens containing the UV stabilizers may he immersed in a dye bath comprising S.O. dye dissolved in a solution of organic solvents such as alcohol, toluene, halogenated hydrocarbon or the like. Other methods of blending the UV stabilizers with the S.O. dye and polymers, such as coating or laminating may also be employed.

One hindered amine light stablizer, useful in the organic photochromic composition of the invention, comprises the structural formula wherein R₁, R₂, R₄, R₅, R₆, R₇, R₉ and R₁₀ are lower alkyl; R₃ and R₈ are lower alkyl or hydrogen; and n = 1 - 12; and in particular, the hindered amine light stabilizer is Bis (2,2,6,6-tetramethyl-4-piperidinyl) sebacate, wherein R₁, R₂, R₄, R₅, R₆, R₇, R₉ and R₁₀ are methyl, R₃ and R₈ are hydrogen, and n = 8, sold under the tradename of Tinuvin 770, and obtained from the Ciba-Geigy Corporation; and also in particular, the hindered amine light stabilizer is Bis (1,2,2,6,6-pentamethyl-4-piperidinyl) sebacate, wherein R₁, R₂ R₄, R₅, R₆, R₇, R₉ and R₁₀ are methyl, R₃ and R₈ are methyl, and n = 8, sold under the tradename of Tinuvin 765, and obtained from the Ciba-Geigy Corporation.

Another hindered amine iight stabilizer which is useful in the organic photochromic composition of the invention comprises the structural formula wherein R₁, ^{R}₂, ^{R}₄, ^{R}₅, ^{R}₆, ^{R}₇, R₉, R₁₀, R₁₁, R₁₂, R₁₃, R₁₄, R₁₅, R₁₆, and R₁₇ are lower alkyl; and R₃ and R₈ are lower alkyl or hydrogen; and in particular, the hindered amine light stabilizer is di(1,2,2,6,6-pentamethyl-4-piperidinyl)-butyl(3',5'-ditertbutyl-4-hydroxybenzyl) malonate, wherein R₁, R₂, R₄, R₅, R₆, R₇, Rg, R₁₀, R₁₂, R₁₃, R₁₄, R₁₅, R₁₆, and R₁₇ are methyl, R₁₁ is butyl, and R₃ and R₈ are methyl, sold under the tradename of Tinuvin 144, and obtained from the Ciba-Geigy Corporation.

Another hindered amine light stabilizer which is useful in the organic photochromic composition of the invention comprises the structural formula wherein R₁, R₄, R₅, R₁₁, and R₁₆ are lower alkyl or hydrogen; R₂, R₃, R₆, R₇, R₈, R₉, R₁₀, R₁₂, R₁₃, R₁₄, R₁₅, R₁₇, and R₁₈ are lower alkyl; n₁ = 1- 12; and n₂ = 1- 15; and in particular, the hindered amine light stabilizer is poly[(6-[(1,1,3,3-tetra-methylbutyl)amino]-1,3,5-triazine-2,4-diyl)(1,6-(2,2,6,6-tetramethyl-4-piperidinyl]amino- hexamethylene)], wherein R₂, R₃, R₆, R₇, R₈, R₉, R₁₀, R₁₂, R₁₃, R₁₄, R₁₅, R₁₇, and R₁₈ are methyl, R₁, R₄, R₅, R₁₁, and R₁₆ are hydrogen, and n₁ = 6, sold under the tradename Chimassorb 944, and obtained from the Ciba-Geigy Corporation.

Another hindered amine light stabilizer which is useful in the organic photochromic composition of the invention comprises the structural formula wherein R₁, R₂, R₄, R₅, Rₛ, R₇, Rg, and R₁₀ are lower alkyl; R₃ and R₈ are lower alkyl or hydrogen; n₁ = 1 - 12; and n₁ = 1 - 15; and in particular, the hindered amine light stabilizer is poly[[6-(morpholino)-s-triazine-2,4-diyl][1,6-(2,2,6,6-tetramethyl-4-piperidyl)amino]hexamethylene], wherein R₁, R₂, R₄, R₅, Rₛ, R₇, R₉, and R₁₀ are methyl, R₃ and R₈ are hydrogen, and n₁ = 6, sold under the tradename Cyasorb 3346, and obtained from the American Cyanamid Corporation.

Another hindered amine light stabilizer which is useful in the organic photochromic composition of the invention comprises the structural formula wherein R₁, R₂, R₃, and R₄ are lower alkyl; and n = 1 - 15; and in particular, the hindered amine light stabilizer is a dimethyl succinate polymer with 4-hydroxy-2,2,6,6-tetramethyl-1-piperidineethanol, wherein R₁, R₂, R₃ and R₄ are methyl, sold under the tradename Tinuvin 622, and obtained from the Ciba-Geigy Corporation.

Other hindered amine light stabilizers which are useful in the organic photochromic composition of the invention include a hindered amine light stabilizer having the structural formula (C₂₆H₅₂N₄)ₙ, wherein n = 1 - -15, sold under the tradename of Spinuvex A-36, and obtained from the Borg-Warner Corporation; and a hindered amine light stabilizer sold under the tradename of Hostavin TMN20, and obtained from the American Hoechst Corporation.

Ultraviolet stabilizers, belonging to the class of excited state quenchers, which are useful in the organic photochromic compound of the invention, include complexes of Ni²+ ion with some organic ligand, cobalt (III) tris-di-n-butyldithiocarbamate, cobalt (II) diisopropyldithiocarbamate (Co DIPDTP), and nickel diisopropyldithiophosphate (Ni DIPDTP).

The preferred excited state quenchers are singlet oxygen quenchers, and in particular, complexes of Ni²⁺ ion with some organic ligand. These Ni²⁺ complexes are normally used in polyolefins to provide protection from photodegradation. Most preferably, the Ni²⁺ complexes are: [2,2'-Thiobis [4-(1,1,3,3-tetramethylbutyl) phenolato] (butylamine)] nickel, having the structural formula sold under the tradename of Cyasorb UV 1084, and obtained from the American Cyanamid Company;

Nickel [0-ethyl (3,5-di-tert-butyl-4-hydroxybenzyl)] phosphonate, having the structural formula sold under the tradename of Irgastab 2002, and obtained from the Ciba-Geigy Corporation; Nickel dibutyldithiocarbamate, having the structural formula sold under the tradename of Rylex NBC, and obtained from E.I. duPont de Nemours & Company;

Bis [2,2'-thiobis-4-(1,1,3,3-tetramethylbutyl) phenolato] nickel, having the structural formula sold under the tradename of UV-Chek AM 101, and obtained from the Ferro Corporation; Nickel di-isopropyl dithiophosphate (Ni DIPDTP), having the structural formula and other Ni²+ complexes sold under the tradenames of UV-Chek AM 105, UV-Chek AM 126, and UV-Chek AM 205 which can also be obtained from the Ferro Corporation.

The preferred S.O. dyes for use in accordance with the invention are 1,3,3,4,5-pentamethyl-9'-methoxy-spiro [indoline-2,3'-[3H]-naphth [2,1-b] [1,4] oxazine;
1,3,3,5,6-pentamethyl-9'-methoxy-spirooxazine;
1,3,3-trimethyl-5'-methoxy spirooxazine;
1,3,3-trimethyl-5-methoxy spirooxazine;
1,3,3,4,5-pentamethyl-8'-bromo spirooxazine;
1,3,3,5,6-pentamethyl-8'-bromo spirooxazine;
1,2,3,3,4,5-hexamethyl-9'-methoxy spirooxazine;
1,2,3,3,5,6-hexamethyl-9'-methoxy spirooxazine;
1,3,3-trimethyl-4-trifluoromethyl-9'-methoxy spirooxaxine;
1,3,3-trimethyl-6-trifluoromethyl-9'-methoxy spirooxazine;
1,3,3-trimethyl-4-trifluoromethyl-5'-methoxy spirooxazine; and
1,3;3-trimethyl-6-trifluoromethyl-5'-methoxy spirooxazine.

The preferred plastic hosts are cellulose acetate butyrate (CAB); CR-39^{TM}, a diethylene glycol bis (allyl carbonate) obtained from PPG Industries, Inc.; Lexan^{TM}, a polycarbonate resin condensation product of bisphenol-A and phosgene, obtained from General Electric; Plèxiglas^{TM}, a polymethyl methacrylate obtained from the Rohm and Haas Company; polyvinyl chloride; and polyolefins.

The invention is further illustrated by the following non-limiting examples.

### Examples 1-8

Eight cellulose acetate butarate (CAB) samples having a thickness of 0,43 - 0,48 mm (17 - 19 mls), containing 0.4 % by weight of a mixture of 1,2,3,3,4,5- and 1,2,3,3,5,6-hexamethyl-9'-methoxy S.O. isomers, with and without hindered amine light stabilizers (HALS) were prepared by casting a methylene chloride solution of CAB. Four successive castings were needed to obtain the desired thickness with good optical appearance. The control sample contained no HALS. The seven other samples contained various hindered amine light stabilizers in an arbitrary amount of 0.4 % by weight. The samples were subjected to a 20-hour cycle Fadeometer exposure testing. After five cycles, the control sample without HALS lost all its photochromism while the samples with HALS still showed good photochromism. The specific HALS used and the percentage of residual photocolorability of the CAB samples after 100 hours of Fadeometer exposure is shown in Table 1.

### Examples 9-10

Two CAB sheet samples (1,52 mm/60 mls) ware made by injection molding. One of the CAB sheet samples had 0.2 % by weight of a mixture of 1,2,3,3,4,5- and 1,2,3,3,5,6-hexamethy)-9'-methoxy spirooxazine isomers and 0.2 % by weight of UV-Chek AM-205 as an excited state quencher. The other sample also had 0.2 % by weight Tinuvin 622 as a hindered amine light stabilizer in addition to the S.O. dye and the UV-Chek AM-205. The sample without the HALS lost all of its photochromism after 15 20-hour Fadeometer exposure cycles. However, the sample with the HALS still had 40 % of the original photocolorability left.

### Examples 11-13

A control sample was cast at 160° in an oven for 20 minutes from a plastisol solution consisting of 31 % diisodecylphthalate, 3 % octyl epoxy tallate, 3 % mark stabilizer, 63 % PVC and 0.1 % 1,3,3,4,5- and 1,3,3,5,6-pentamethyl-9'-methoxy S.O. dye mixture. Two more samples were prepared as follows: One sample had, in addition to the ingredients in the control sample, 0.2 % by weight UV-Chek AM-205, and the other sample had 0.2 % by weight UV-Chek AM-205 and 1.0 % by weight Tinuvin 622. The control sample lost all of its photochromic effect after 20 hours of Fadeometer exposure; the sample with UV-Chek AM-205 lasted 80 hours before losing its photochromic effect, and the sample with both UV-Chek AM-205 and Tinuvin 622 lasted 180 hours before losing its photochromic effect.

### Examples 14-18

An ethanol solution of 1,3,3-trimethyl S.O. dye was prepared by dissolving 13.1 mg of dye in 100.0 ml of ethanol. Two milliters of the solution was placed in each of five 10.0 ml volumetric flasks. Then, 0.01 ml of 1 N HCI was added to each flask and each solution was diluted with ethanol to 10.0 ml. Each solution was originally colorless but became pinkish and lost its photochromic effect once the HCI was added. To four of the solutions was added about 3 mg of either Tinuvin 770, Tinuvin 765, Cyasorb 1084 or UV-Chek AM-205. The solutions containing the Tinuvin and Cyasorb compounds reverted to colorless solutions and regained their photochromic effect, while the other solutions remained pinkish and showed no photochromic effect.

## Claims (Claims for the following Contracting State(s) : s: BE, CH, DE, FR, GB, IT, LI, LU, NL, SE)

1. A method of increasing the light fatigue resistance of a spirooxazine photochromic composition which comprises incorporating in said composition a hindered amine light stabilizer.

2. A method according to claim 1 wherein said photochromic composition additionally contains a singlet oxygen quencher ultraviolet stabilizer.

3. A method according to claim 2 wherein said singlet oxygen quencher ultraviolet stabilizer is a Ni²⁺ ion complex with an organic liqand.

4. A method according to claim 2 wherein said singlet oxygen quencher ultraviolet stabilizer is selected from [2,2'-thiobis [4-(1,1,3,3-tetramethylbutyl) phenolato] (butylamine)] nickel, nickel [0-ethyl (3,5-di-tert-butyl-4-hydroxybenzyl)] phosphonate, nickel dibutyldithiocarbamate, nickel di-isopropyl dithiophosphate, bis [2,2'-thiobis-4-(1,1,3,3-tetramethylbutyl) phenolato] nickel, cobalt (111) tris-di-n-butyldithiocarbamate, and cobalt (II) diisopropyldithiocarbamate.

5. A method according to one of claims 1 to 4, wherein said photochromic composition comprises a polymer cointaining about 0.1 % to about 15 % by weight spriooxazine photochromic dye.

6. A method according to claim 5 wherein said hindered amine light stabilizer and said singlet oxygen quencher ultraviolet stabilizer are incorporated in said photochromic composition in a total amount of about 0.01 % to about 5 % by weight.

7. A method according to claim 6 wherein said hindered amine light stabilizer is a tetramethyl peridine derivative.

8. A method according to one of claims 1 to 6 wherein said hindered amine light stabilizer is selected from one or more compounds of the following formulae: wherein Ri, R₂, R₄, R₅, R₆, R₇, Rg, and R₁₀ are alkyl having 1 to 12 carbon atoms, R₃ and R₈ are selected from alkyl having 1 to 12 carbon atoms and hydrogen, and n is 1 -12; wherein R₁, R₂, R₄, R₅, R₆, R₇, Rg, R₁₀, R₁₁, R₁₂, R₁₃, R₁₄, R₁₅, R₁₆ and R₁₇ are alkyl having 1 to 12 carbon atoms, and R₃ and R₈ are selected from alkyl having 1 to 12 carbon atoms and hydrogen, wherein R₁, R₄, R₅ R₁₁ and R₁₆ are selected from alkyl having 1 to 12 carbon atoms and hydrogen R₂, R₃, R₇, R₈, Rg, R₁₀, R₁₂, R₁₃, R₁₄, R₁₅, R₁₇ and R₁₈ are alkyl having 1 to 12 carbon atoms; n₁ is 1 - 12, and n₂ is 1 - 15; wherein R₁, R₂, R₄, R₅, R₆, R₇, Rg, and R₁₀ are alkyl having 1 to 12 carbon atoms, R₃ and R_{B} are selected from alkyl having 1 to 12 carbon atoms and hydrogen, n₁ is 1 - 12 and n₂ is 1 - 15; wherein R₁, R₂, R₃, and R₄ are alkyl having 1 to 12 carbon atoms, and n is 1 - 15; and (C₂₆ H₅₂ N₄)ₙ wherein n is 1 - 15.

9. A method according to claim 8 wherein said photochromic composition contains one or more of a spiroaxazine photochromic dye of the formula wherein one of R₁, R₂ and R₃ is selected from the group consisting of hydrogen, halogen, alkoxy having 1 to 12 carbon atoms, and alkyl having 1 to 12 carbon atoms and the others are hydrogen; R₄ and R₅ are selected from the group consisting of hydrogen, alkyl having 1 to 12 carbon atoms, alkoxy having 1 to 12 carbon atoms, halogen, and trifluoromethyl; and R₆ is alkyl having 1 to 12 carbon atoms.

10. A method according to claim 9 wherein said hindered amine light stabilizer is selected from one or more of
bis (2,2,6,6-tetramethyl-4-piperidinyl) sebacate;
bis (1,2,2,6,6-pentamethyl-4-piperidinyl) sebacate;
di(1,2,2,6,6-pentamethyl-4-piperidinyl) - butyl(3',5'-ditertbutyl-4-hydroxybenzyl) malonate;
poly[(6-[(1,1,3,3-tetramethylbutyl) - amino] -1,3,5-triazine-2,4-diyl) (1,6-[2,2,6,6-tetramethyl-4-piperidinyl] amino- hexamethylene)]; poly[[6-(morpholino)-s-triazine-2,4-diyl] [1,6-(2,2,6,6-tetramethyl-4-piperidyl) amino] -hexamethylene];
and dimethyl succinate polymer with 4-hydroxy-2,2,6,6-tetramethyl-1-piperidineethanol.

11. A spiro oxazine photochromic composition into which a hindered amine light stabilizer is incorporated.

12. A photochromic composition according to claim 11 comprising at least one photochromic compound having the structural formula wherein one of R₁, R₂ and R₃, is selected from the group consisting of hydrogen, halogen, alkoxy having 1 to 12 carbon atoms, and alkyl having 1 to 12 carbon atoms and the others are hydrogen; R₄ and R₅ are selected from the group consisting of hydrogen, alkyl having 1 to 12 carbon atoms, alkoxy having 1 to 12 carbon atoms, halogen, and trifluoromethyl; and R₆ is alkyl having 1 to 12 carbon atoms, and a hindered amine light stabilizer.

13. A composition according to claim 11 additionally comprising a singlet oxygen quencher ultraviolet stabilizer.

14. A composition according to claim 13 wherein said singlet oxygen quencher ultraviolet stabilizer is a Ni²+ ion complex with an organic ligand.

15. A composition according to claim 13 wherein said singlet oxygen quencher ultraviolet stabilizer is selected from [2,2'-thiobis [4-(1,1,3,3-tetramethylbutyl) phenolato] (butylamine)] nickel, nickel-[0-ethyl (3,5-di- tert-butyl-4-hydroxybenzyl)] phosphonate, nickel dibutyldithiocarbamate, nickel di-isopropyl dithiophosphate, bis [2,2'-thiobis-4-(1,1,3,3-tetramethylbutyl) phenolato] nickel, cobalt (III) tris-di-n-butyldithiocarbamate, and cobalt (II) diisopropyldithiocarbamate.

16. A composition according to one of claims 11 to 15 wherein said hindered amine light stabilizer is selected from one or more compounds of the following formulae: wherein R₁, R₂, R₄, R₅, R₆, R₇, R₉, and R₁₀ are alkyl having 1 to 12 carbon atoms, R₃ and R₈ are selected from alkyl having 1 to 12 carbon atoms and hydrogen, and n is 1 - 12; wherein R₁, R₂, R₄, R₅, R₆, R₇, Rg, R₁₀, R₁₁, R₁₂, R₁₃, R₁₄, R₁₅, R₁₆ and R₁₇ are alkyl having 1 to 12 carbon atoms, and R₃ and R₈ are selected from alkyl having 1 to 12 carbon atoms and hydrogen; wherein R₁, R₄, R₅, R₁₁ and R₁₆ are selected from alkyl having 1 to 12 carbon atoms and hydrogen R₂, R₃, R₇, R₈, R₉, R₁₀, R₁₂, R₁₃, R₁₄, R₁₅, R₁₇ and R₁₈ are alkyl having 1 to 12 carbon atoms; n₁ is 1 - 12, and n₂ is 1 - 15; wherein R₁, R₂, R₄, R₅, R₆, R₇, R₉, and R₁₀ are alkyl having 1 to 12 carbon atoms, R₃ and R₈ are selected from alkyl having 1 to 12 carbon atoms and hydrogen, n₁ is 1 - 12 and n₂ is 1 - 15; wherein R₁, R₂, R₃, and R₄ and alkyl having 1 to 12 carbon atoms, and n is 1 - 15; and (C₂₆H₅₂N₄)ₙ wherein n is 1 - 15.

17. A composition according to claim 16 wherein said hindered amine light stabilizer is selected from one or more of
bis (2,2,6,6-tetramethyl-4-piperidinyl) sebacate;
bis (1,2,6,6,-pentamethyl-4-piperidinyl) sebacate;
di(1,2,2,6,6-pentamethyl-4-piperidinyl) - butyl(3',5'-ditertbutyl-4-hydroxybenzyl) malonate; poly[(6-[(1,1,3,3-tetramethylbutyl) - amino]-1,3,5-triazine-2,4-diyl) (1,6-[2,2,6,6-tetramethyl-4-piperidinyl] amino- hexamethylene)]; poly[[6-(morpholino)-s-triazine-2,4-diyl] [1,6-(2,2,6,6-tetramethyl-4-piperidyl) amino] -hexamethylene] ;
and dimethyl succinate polymer with 4-hydroxy-2,2,6,6-tetramethyl-1-piperidineethanol.

18. A composition according to claim 16 additionally comprising a plastic host.

19. A composition according to claim 18 containing about 0.1 % to about 15 % by weight of said photochromic compound and about 0.01 % to about 5 % by weight of said stabilizer or stabilizers.

## Claims (Claims for the following Contracting State(s) : Austria)

1. A method of increasing the light fatigue resistancc of a spirooxazine photochromic composition which comprises incorporating in said composition a hindered amine light stabilizer.

2. A method according to claim 1 wherein said photochromic composition additionally contains a singlet oxygen quencher ultraviolet stabilizer.

3. A method according to claim 2 wherein said singlet oxygen quencher ultraviolet stabilizer is a Ni²⁺ ion complex with an organic liqand.

4. A method according to claim 2 wherein said singlet oxygen quencher ultraviolet stabilizer is selected from [2,2' -thiobis [4-(1,1,3,3-tetramethylbutyl) phenolato] (butylamine)] nickel, nickel [0-ethyl (3,5-di-tert-butyl-4-hydroxybenzyl)] phosphonate, nickel dibutyldithiocarbamate, nickel di-isopropyl dithiophosphate, bis [2,2'-thiobis-4-(1,1,3,3-tetramethylbutyl) phenolato] nickel, cobalt (III) tris-di-n-butyldithiocarbamate, and cobalt (II) diisopropyldithiocarbamate.

5. A method acccording to one of claims 1 to 4, wherein said photochromic composition comprises a polymer containing about 0.1 % to about 15 % by weight spriooxazine photochromic dye.

6. A method according to claim 5 wherein said hindered amine light stabilizer and said singlet oxygen quencher ultraviolet stabilizer are incorporated in said photochromic composition in a total amount of about 0.01 % to about 5 % by weight.

7. A method according to claim 6 wherein said hindered amine light stabilizer is a tetramethyl piperidine derivative.

8. A method according to one of claims 1 to 6 wherein said hindered amine light stabilizer is selected from one or more compounds of the following formulae: wherein R₁, R₂, R₄, R₅, R₆, R₇, R₉, and R₁₀ alkyl having 1 to 12 carbon atoms, R₃ and R₈ are selected from alkyl having 1 to 12 carbon atoms and hydrogen, and n is 1 - 12; wherein R₁, ^{R}₂, ^{R}₄, ^{R}₅, ^{R}₆, ^{R}₇, Rg, R₁₀, R₁₁, R₁₂, R₁₃, R₁₄, R₁₅, R₁₆ and R₁₇ are alkyl having 1 to 12 carbon atoms, and R₃ and R₈ are selected from alkyl having 1 to 12 carbon atoms and hydrogen; wherein R₁, R₄, R₅, R₁₁ and R₁₆ are selected from alkyl having 1 to 12 carbon atoms and hydrogen, R₂, R₃, R₇, R₈, Rs, R₁₀, R₁₂, R₁₃, R₁₄, R₁₅, R₁₇ and R₁₈ are alkyl having 1 to 12 carbon atoms; n₁ is 1 -12, and n₂ is 1 - 15; wherein R₁, R₂, R₄, R₅, R₆, R₇, R₉, and R₁₀ are alkyl having 1 to 12 carbon atoms, R₃ and R₈ are selected from alkyl having 1 to 12 carbon atoms and hydrogen, n₁ is 1 - 12 and n₂ is 1 - 15; wherein R₁, R₂, R₃, and R₄ are alkyl having 1 to 12 carbon atoms, and n is 1 - 15; and (C₂₆H₅₂N₄)ₙ wherein n is 1 - 15.

9. A method according to claim 8 wherein said photochromic composition contains one or more of a spiroaxazine photochromic dye of the formula wherein one of R₁, R₂ and R₃ is selected from the group consisting of hydrogen, halogen, alkoxy having 1 to 12 carbon atoms, and alkyl having 1 to 12 carbon atoms and the others are hydrogen; R₄ and R₅ are selected from the group consisting of hydrogen, alkyl having 1 to 12 carbon atoms, alkoxy having 1 to 12 carbon atoms, halogen, and trifluoromethyl; and R₆ is alkyl having 1 to 12 carbon atoms.

10. A method according to claim 9 wherein said hindered amine light stabilizer is selected from one or more of
bis (2,2,6,6-tetramethyl-4-piperidinyl) sebacate;
bis (1,2,2,6,6-pentamethyl-4-piperidinyl) sebacate;
di(1,2,2,6,6-pentamethyl-4-piperidinyl) - butyl(3',5'-ditertbutyl-4-hydroxybenzyl) malonate; poly[(6-[(1,1,3,3-tetramethylbutyl) - amino] -1,3,5-triazine-2,4-diyl) (1,6-[2,2,6,6-tetramethyl-4-piperidinyl] amino- hexamethylene)]; poly[[6-(morpholino) -s-triazine-2,4-diyl] [1,6-(2,2,6,6-tetramethyl-4-piperidyl) amino] -hexamethylene];
and dimethyl succinate polymer with 4-hydroxy-2,2,6,6-tetramethyl-1-piperidineethanol.

11. A method according to claim 8 additionally comprising a plastic host.

12. A method according to claim 11 containing about 0.1 % to about 15 % by weight of said photochromic compound and about 0.01 % to about 5 % by weight of said stabilizer or stabilizers.

## Patentansprüche (Patentansprüche für folgende(n) Vertragsstaat(en) : BE, CH, DE, FR, GB, IT, LI, LU, NL und SE)

1. Verfahren zum Erhöhen der Lichtermüdungsbeständigkeit eines photochromen spirooxazinhaltigen Gemisches, dadurch gekennzeichnet, daß in das Gemisch ein Lichtstabilisator in Form eines gehinderten Amins eingearbeitet wird.

2. Verfahren nach Anspruch 1, worin das photochrome Gemisch zusätzlich einen UV-Stabilisator in Form eines Singulett-Sauerstoff-Löschers enthält.

3. Verfahren nach Anspruch 2, worin der UV-Stabilisator in Form eines Singulett-Sauerstoff-Löschers ein Ni2+-lonenkomplex mit einem organischen Liganden ist.

4. Verfahren nach Anspruch 2, worin der UV-Stabilisator in Form eines Singulett-Sauerstoff-Löschers aus den Verbindungen [2,2'-Thiobis-[4-(1,1,3,3-tetramethylbutyl)-phenolato]-(butylamin)]-nickel, Nickel-[0-ethyl-(3,5-di-tert.-butyl-4-hydroxybenzyl)]-phosphonat, Nickeldibutyldithiocarbamat, Nickeldiisopropyldithiophosphat, Bis-(2,2'-thiobis-4-(1,1,3,3-tetramethylbutyl)-phenolato]-nickel, Cobalt(III)-tris-di-n-butyldithiocarbamat und Cobalt(II)-diisopropyldithiocarbamat ausgewählt ist.

5. Verfahren nach einem der Ansprüche 1 bis 4, worin das photochrome Gemisch ein Polymer enthält, das etwa 0,1 bis etwa 15 Gew.-% eines photochromen Spirooxazin-Farbstoffs aufweist.

6. Verfahren nach Anspruch 5, worin der Lichtstabilisator in Form eines gehinderten Amins und der UV-Stabilisator in Form des Singulett-Sauerstoff-Löschers in das photochrome Gemisch in einer Gesamtmenge von etwa 0,01 bis etwa 5 Gew.-% eingearbeitet werden.

7. Verfahren nach Anspruch 6, worin der Lichtstabilisator in Form eines gehinderten Amins ein Tetramethylpiperidinderivat ist.

8. Verfahren nach einem der Ansprüche 1 bis 8, worin der Lichtstabilisator in Form eines gehinderten Amins aus einer oder mehreren Verbindungen der folgenden Formeln worin R_{1,} R₂, R₄, R₅, R₆, R₇, R₉ und R₁₀ jeweils einen Alkylrest mit 1 bis 12 Kohlenstoffatomen bedeuten sowie R₃ und R₈ aus der Gruppe ausgewählt sind, die aus Alkylresten mit 1 bis 12 Kohlenstoffatomen und Wasserstoff besteht, sowie n eine Zahl von 1 bis 12 bedeutet, worin R₁, R₂, ^{R}₄, ^{R}₅, R₆, R₇, R₉, R₁₀, R₁₁, R₁₂, R₁₃, R₁₄, R₁₅, R₁₆ und R₁₇ jeweils einen Alkylrest mit 1 bis 12 Kohlenstoffatomen bedeuten und R₃ und R₈ aus der Gruppe ausgewählt sind, die aus Alkylresten mit 1 bis 12 Kohlenstoffatomen und Wasserstoff besteht, worin R₁, R₄, R₅, R₁₁ und R₁₆ aus der Gruppe ausgewählt ist, die aus Alkylresten mit 1 bis 12 Kohlenstoffatomen und Wasserstoff besteht, sowie ^{R}₂, ^{R}₃, R₇, R₈, R₉, R₁₀, R₁₂, R₁₃, R₁₄, R₁₅, R₁₇ und R₁₈ jeweils einen Alkylrest mit 1 bis 12 Kohlenstoffatomen bedeuten sowie n₁ eine Zahl von 1 bis 12 und n₂ eine Zahl von 1 bis 15 darstellen, worin R₁, R₂, R₄, R₅, R₆, R₇, R₉ und R₁₀ jeweils einen Alkylrest mit 1 bis 12 Kohlenstoffatomen bedeuten sowie R₃ und R₈ aus der Gruppe ausgewählt sind, die aus Alkylresten mit 1 bis 12 Kohlenstoffatomen und Wasserstoff besteht, sowie n₁ eine Zahl von 1 bis 12 und n₂ eine Zahl von 1 bis 15 darstellen, worin R₁, R₂, R₃ und R₄ jeweils Alkylreste mit 1 bis 12 Kohlenstoffatomen bedeuten sowie n eine Zahl von 1 bis 15 darstellt, und
(C₂₆H₅₂N₄)ₙ, worin n eine Zahl von 1 bis 15 bedeutet,
ausgewählt wird.

9. Verfahren nach Anspruch 8, worin das photochrome Gemisch einen oder mehrere photochrome Spirooxazin-Farbstoffe der Formel enthält, worin einer der Reste R₁, R₂ und R₃ aus der Gruppe ausgewählt ist, die aus Wasserstoff, Halogen, Alkoxyresten mit 1 bis 12 Kohlenstoffatomen und Alkylresten mit 1 bis 12 Kohlenstoffatomen besteht, und die anderen dieser Reste Wasserstoffatome darstellen, R₄ und R₅ aus der Gruppe ausgewählt sind, die aus Wasserstoff, Alkylresten mit 1 bis 12 Kohlenstoffatomen, Alkoxyresten mit 1 bis 12 Kohlenstoffatomen, Halogen und der Trifluormethylgruppe besteht, sowie R₆ einen Alkylrest mit 1 bis 12 Kohlenstoffatomen bedeutet.

10. Verfahren nach Anspruch 9, worin der Lichtstabilisator in Form eines gehinderten Amins aus einer oder mehreren der Verbindungen Bis-(2,2,6,6-tetramethyl-4-piperidinyl)-sebacat, Bis-(1,2,2,6,6-pentamethyl-4-piperidinyl)-sebacat, Di-(1,2,2,6,6-pentamethyl-4-piperidinyl)-butyl-(3',5'-di-tert.-butyl-4-hydroxybenzyl)-malonat, Poly-[(6- [(1,1,3,3-tetramethylbutyl)-amino]-1,3,5-triazin-2,4-diyl)-(1,6-(2,2,6,6-tetramethyl-4-piperidinyl]-aminohexamethylen)], Poly- {[6-(morpholino)-s-triazin-2,4-diyl]-[1,6-(2,2,6,6-tetramethy)-4-piperidyl)-amino]-hexamethylen} und Dimethylsuccinatpolymer mit 4-Hydroxy-2,2,6,6-tetramethyl-1-piperidinethanol ausgewählt wird.

11. Photochromes spirooxazinhaltiges Gemisch, in das ein Lichtstabilisator in Form eines gehinderten Amins eingearbeitet ist.

12. Photochromes Gemisch nach Anspruch 11, enthaltend mindestens eine photochrome Verbindung der Strukturformel worin einer der Reste R₁, R₂ und R₃ aus der Gruppe ausgewählt ist, die aus Wasserstoff, Halogen, Alkoxyresten mit 1 bis 12 Kohlenstoffatomen und Alkylresten mit 1 bis 12 Kohlenstoffatomen besteht, und die anderen dieser Reste Wasserstoffatome darstellen, R₄ und R₅ aus der Gruppe ausgewählt sind, die aus Wasserstoff, Alkylresten mit 1 bis 12 Kohlenstoffatomen, Alkoxyresten mit 1 bis 12 Kohlenstoffatomen, Halogen und der Trifluormethylgruppe besteht, und R₆ einen Alkylrest mit 1 bis 12 Kohlenstoffatomen bedeutet, sowie einen Lichtstabilisator in Form eines gehinderten Amins.

13. Gemisch nach Anspruch 11, das zusätzlich einen UV-Stabilisator in Form eines Singulett-Sauerstoff-Löschers enthält.

14. Gemisch nach Anspruch 13, worin der UV-Stabilisator in Form eines Singulett-Sauerstoff-Löschers ein Ni²+-lonenkomplex mit einem organischen Liganden ist.

15. Gemisch nach Anspruch 13, worin der UV-Stabilisator in Form eines Singulett-Sauerstoff-Löschers aus den Verbindungen {2,2'-Thiobis-[4-(1,1,3,3-tetramethylbutyl)-phenolato]-(butylamin)}-nickel, Nickel-[0-ethyl-(3,5-di-tert.-butyl-4-hydroxybenzyl)]-phosphonat, Nickeldibutyldithiocarbamat, Nickeldiisopropyldithiophosphat, Bis-[2,2'-thiobis-4-(1,1,3,3-tetramethylbutyl)-phenolato]-nickel, Cobalt(III)-tris-di-n-butyldithiocarbamat und Cobalt(II)-diisopropyldithiocarbamat ausgewählt ist.

16. Gemisch nach einem der Ansprüche 11 bis 15, worin der Lichtstabilisator in Form eines gehinderten Amins aus einer oder mehreren Verbindungen der folgenden Formeln worin R₁, R₂, R₄, R₅, Ro R₇ R₉ und R₁₀ jeweils einen Alkylrest mit 1 bis 12 Kohlenstoffatomen bedeuten sowie R₃ und R₈ aus der Gruppe ausgewählt sind, die aus Alkylresten mit 1 bis 12 Kohlenstoffatomen und Wasserstoff besteht, sowie n eine Zahl von 1 bis 12 bedeutet, worin R₁, ^{R}₂, R₄, R₅, R₆, R₇, R₉, R₁₀, R₁₁, R₁₂, R₁₃, R₁₄, R₁₅, R₁₆ und R₁₇ jeweils einen Alkylrest mit 1 bis 12 Kohlenstoffatomen bedeuten und R₃ und R₈ aus der Gruppe ausgewählt sind, die aus Alkylresten mit 1 bis 12 Kohlenstoffatomen und Wasserstoff besteht, worin R₁, R₄, R₅, R₁₁ und R₁₆ aus der Gruppe ausgewählt sind, die aus Alkylresten mit 1 bis 12 Kohlenstoffatomen und Wasserstoff besteht, sowie R₂, R₃, R₇, R₈, R₉, R₁₀, R₁₂, R₁₃, R₁₄, R₁₅, R₁₇ und R₁₈ jeweils einen Alkylrest mit 1 bis 12 Kohlenstoffatomen bedeuten sowie n₁ eine Zahl von 1 bis 12 und n₂ eine Zahl von 1 bis 15 darstellen, worin R₁, R₂, R₄, R₅, R₆, R₇, R₉ und R₁₀ jeweils ein Alkylrest mit 1 bis 12 Kohlenstoffatomen bedeuten sowie R₃ und R₈ aus der Gruppe ausgewählt sind, die aus Alkylresten mit 1 bis 12 Kohlenstoffatomen und Wasserstoff besteht, sowie n₁ eine Zahl von 1 bis 12 und n₂ eine Zahl von 1 bis 15 darstellen, worin R₁, R₂, R₃ und R₄ jeweils Alkylreste mit 1 bis 12 Kohlenstoffatomen bedeuten sowie n eine Zahl von 1 bis 15 darstellt, und
(C₂₆H₅₂N₄)ₙ worin n eine Zahl von 1 bis 15 bedeutet,
ausgewählt wird.

17. Gemisch nach Anspruch 16, worin der Lichtstabilisator in Form eines gehinderten Amins aus einer oder mehreren der Verbindungen Bis-(2,2,6,6-tetramethyl-4-piperidinyl)-sebacat, Bis-(1,2,2,6,6-pentamethyl-4-piperidinyl)-sebacat, Di-(1,2,2,6,6-pentamethyl-4-piperidinyl)-butyl-(3',5'-di-tert.-butyl-4-hydroxybenzyl)-malonat, Poly-[(6-[(1,1,3,3-tetramethylbutyl)-amino]-1,3,5-triazin-2,4-diyl]-(1,6-[2,2,6,6-tetramethyl-4-piperidinyl]-aminohexamethylen)], Poly- {[6-(morpho)ino-s-triazin-2,4-diyl]-[1,6-(2,2,6,6-tetramethyl-4-piperidyl)-amino]-hexamethylen und Dimethylsuccinatpolymer mit 4-Hydroxy-2,2,6,6-tetramethyl-1-piperidinethanol ausgewählt ist.

18. Gemisch nach Anspruch 16, das zusätzlich einen Wirt aus Kunststoff enthält.

19. Gemisch nach Anspruch 18, das etwa 0,1 bis etwa 15 Gew.-% der photochromen Verbindung und etwa 0,01 bis etwa 5 Gew.-% des Stabilisators oder der Stabilisatoren enthält.

## Patentansprüche (Patentansprüche für folgende(n) Vertragsstaat(en) : AT)

1. Verfahren zum Erhöhen der Lichtermüdungsbeständigkeit eines photochromen spirooxazinhaltigen Gemisches, dadurch gekennzeichnet, daß in das Gemisch ein Lichtstabilisator in Form eines gehinderten Amins eingearbeitet wird.

2. Verfahren nach Anspruch 1, worin das photochrome Gemisch zusätzlich einen UV-Stabilisator in Form eines Singulett-Sauerstoff-Löschers enthält.

3. Verfahren nach Anspruch 2, worin der UV-Stabilisator in Form eines Singulett-Sauerstoff-Löschers ein Ni²+-lonenkomplex mit einem organischen Liganden ist.

4. Verfahren nach Anspruch 2, worin der UV-Stabilisator in Form eines Singulett-Sauerstoff-Löschers aus den Verbindungen [2,2'-Thiobis-[4-(1,1,3,3-tetramethylbutyl)-phenolato]-(butylamin)]-nickel, Nickel-[0-ethyl-(3,5-di-tert.-butyl-4-hydroxybenzyl)]-phosphonat, Nickeldibutyldithiocarbamat, Nickeldiisopropyldithiophosphat, Bis-[2,2'-thiobis-4-(1,1,3,3-tetramethylbutyl)-phenolato]-nickel, Cobalt(III)-tris-di-n-butyldithiocarbamat und Cobatt(II)-diisopropyldithiocarbamat ausgewählt ist.

5. Verfahren nach einem der Ansprüche 1 bis 4, worin das photochrome Gemisch ein Polymer enthält, das etwa 0,1 bis etwa 15 Gew.-% eines photochromen Spirooxazin-Farbstoffs aufweist.

6. Verfahren nach Anspruch 5, worin der Lichtstabilisator in Form eines gehinderten Amins und der UV-Stabilisator in Form des Singulett-Sauerstoff-Löschers in das photochrome Gemisch in einer Gesamtmenge von etwa 0,01 bis etwa 5 Gew.-% eingearbeitet werden.

7. Verfahren nach Anspruch 6, worin der Lichtstabilisator in Form eines gehinderten Amins ein Tetramethylpiperidinderivat ist.

8. Verfahren nach einem der Ansprüche 1 bis 6, worin der Lichtstabilisator in Form eines gehinderten Amins aus einer oder mehreren Verbindungen der folgenden Formeln worin R₁, R₂, R₄, R₅, R₆, R₇, R₉ und R₁₀ jeweils einen Alkylrest mit 1 bis 12 Kohlenstoffatomen bedeuten sowie R₃ und R₈ aus der Gruppe ausgewählt sind, die aus Alkylresten mit 1 bis 12 Kohlenstoffatomen und Wasserstoff besteht, sowie n eine Zahl von 1 bis 12 bedeutet, worin R₁, ^{R}₂, R₄, R₅, R₆, R₇, R₉, R₁₀, R₁₁, R₁₂, R₁₃, R₁₄, R₁₅, R₁₆ und R₁₇ jeweils einen Alkylrest mit 1 bis 12 Kohlenstoffatomen bedeuten und R₃ und R₈ aus der Gruppe ausgewählt sind, die aus Alkylresten mit 1 bis 12 Kohlenstoffatomen und Wasserstoff besteht, worin R₁, R₄, R₅, R₁₁ und R₁₆ aus der Gruppe ausgewählt ist, die aus Alkylresten mit 1 bis 12 Kohlenstoffatomen und Wasserstoff besteht, sowie ^{R}₂, R₃, R₇, R₈, Rg, R₁₀, R₁₂, R₁₃, R₁₄, R₁₅, R₁₇ und R₁₈ jeweils einen Alkylrest mit 1 bis 12 Kohlenstoffatomen bedeuten sowie n₁ eine Zahl von 1 bis 12 und n₂ eine Zahl von 1 bis 15 darstellen, worin R₁, R₂, R₄, R₅, R₆, R₇, R₉ und R₁₀ jeweils einen Alkylrest mit 1 bis 12 Kohlenstoffatomen bedeuten sowie R₃ und R₈ aus der Gruppe ausgewählt sind, die aus Alkylresten mit 1 bis 12 Kohlenstoffatomen und Wasserstoff besteht, sowie n₁ eine Zahl von 1 bis 12 und n₂ eine Zahl von 1 bis 15 darstellen, worin Rₗ, R₂, R₃ und R₄ jeweils Alkylreste mit 1 bis 12 Kohlenstoffatomen bedeuten sowie n eine Zahl von 1 bis 15 darstellt, und
(C₂₆H₅₂N₄)ₙ, worin n eine Zahl von 1 bis 15 bedeutet,
ausgewählt wird.

9. Verfahren nach Anspruch 8, worin das photochrome Gemisch einen oder mehrere photochrome Spirooxazin-Farbstoffe der Formel enthält, worin einer der Reste R₁, R₂ und R₃ aus der Gruppe ausgewählt ist, die aus Wasserstoff, Halogen, Alkoxyresten mit 1 bis 12 Kohlenstoffatomen und Alkylresten mit 1 bis 12 Kohlenstoffatomen besteht, und die anderen dieser Reste Wasserstoffatome darstellen, R₄ und R₅ aus der Gruppe ausgewählt sind, die aus Wasserstoff, Alkylresten mit 1 bis 12 Kohlenstoffatomen, Alkoxyresten mit 1 bis 12 Kohlenstoffatomen, Halogen und der Trifluormethylgruppe besteht, sowie R₆ einen Alkylrest mit 1 bis 12 Kohlenstoffatomen bedeutet.

10. Verfahren nach Anspruch 9, worin der Lichtstabilisator in Form eines gehinderten Amins aus einer oder mehreren der Verbindungen Bis-(2,2,6;6-tetramethyl-4-piperidinyl)-sebacat, Bis-(1,2,2,6,6-pentamethyl-4-piperidinyl)-sebacat, Di-(1,2,2,6,6-pentamethyl-4-piperidinyl)-butyl-(3',5'-di-tert.-butyl-4-hydroxybenzyl)-malonat, Poly-[(6- [(1,1,3,3-tetramethylbutyl)-amino]-1,3,5-triazin-2,4-diyl)-(1,6-2,2,6,6-tetramethyl-4-piperidinyl]-aminohexamethylen)], Poly- {[6-(morpho)ino-s-triazin-2,4-diyl]-[1,6-(2,2,6,6-tetramethyl-4-piperidyl)-amino]-hexamethylen} und Dimethylsuccinatpolymer mit 4-Hydroxy-2,2,6,6-tetramethyl-1-piperidinethanol ausgewählt wird.

11. Verfahren nach Anspruch 8, bei dem zusätzlich ein Wirt aus Kunststoff eingesetzt wird.

12. Verfahren nach Anspruch 11, bei dem etwa 0,1 bis etwa 15 Gew.-% der photochromen Verbindung und etwa 0,01 bis etwa 5 Gew.-% des Stabilisators oder der Stabilisatoren eingesetzt werden.

## Revendications (Revendications pour l'(les) Etat(s) contractant(s) suivant(s) : BE, CH, DE, FR, GB, IT, LI, LU, NL, SE)

1. Procédé en vue d'accroître la résistance à la fatigue à la lumière d'une composition photochrome de spiro- oxazine, caractérisé en ce qu'il consiste à incorporer, dans cette composition, un stabilisant à la lumière à base d'une amine à empêchement stérique.

2. Procédé selon la revendication 1, caractérisé en ce que cette composition photochrome contient, en outre, un stabilisant extincteur d'oxygène singulet contre l'ultraviolet.

3. Procédé selon la revendication 2, caractérisé en ce que le stabilisant extincteur d'oxygène singulet contre l'ultraviolet est un complexe d'ions Ni²+ avec un coordinat organique.

4. Procédé selon la revendication 2, caractérisé en ce que le stabilisant extincteur d'oxygène singulet contre l'ultraviolet est choisi parmi le [2,2'-thiobis-(4-(1,1,3,3-tétraméthylbutyl)phénolato]-(butylamine)]nickel, le [0- éthyl-(3,5-di-tert.-butyl-4-hydroxybenzyl)]phosphonate de nickel, le dibutyldithiocarbamate de nickel, le diisopropyl-dithiophosphate de nickel, le bis-[2,2'-thiobis-4-(1,1,3,3-tétraméthylbutyl)-phénolato]nickel, le tris-di-n-butyldithiocarbamate de cobalt(III) et le diisopropyldithiocarbamate de cobalt(II).

5. Procédé selon une des revendications 1 à 4, caractérisé en ce que la composition photochrome comprend un polymère contenant environ 0,1 à environ 15 % en poids d'un colorant photochrome de spiro-oxazine.

6. Procédé selon la revendication 5, caractérisé en ce que le stabilisant vis-à-vis de la lumière à base d'une amine à empêchement stérique et le stabilisant extincteur d'oxygène singulet contre l'ultraviolet sont incorporés dans la composition photochrome en une quantité totale d'environ 0,01 % à environ 5 % en poids.

7. Procédé selon la revendication 6, caractérisé en ce que le stabilisant contre la lumière à base d'une amine à empêchement stérique est un dérivé de la tétraméthyl-pipéridine.

8. Procédé selon une des revendications 1 à 6, caractérisé en ce que le stabilisant vis-à-vis de la lumière à base d'une amine à empêchement stérique est choisi parmi un ou plusieurs composés repondant aux formules suivantes: où R₁, R₂, R₄, R₅, R₆, R₇, R₉ et R₁₀ sont des groupes alkyle contenant 1 à 12 atomes de carbone, R₃ et R₈ sont choisis parmi les groupes alkyle contenant 1 à 12 atomes de carbone, et l'atome d'hydrogène, tandis que n'est égal à 1 - 12; où R₁, R₂, R₄, R₅, R₆, R₇, Rg, R₁₀, R₁₁, R₁₂, R₁₃, R₁₄, R₁₅, R₁₆ et R₁₇ sont des groupes alkyle contenant 1 à 12 atomes de carbone, tandis que R₃ et R₈ sont choisis parmi les groupes alkyle contenant 1 à 12 atomes de carbone, et l'atome d'hydrogène; où R₁, R₄, R₅, R₁₁ et R₁₆ sont choisis parmi les groupes alkyle contenant 1 à 12 atomes de carbone, ainsi que l'atome d'hydrogène, R₂, R₃, R₇, R₈, R₉, R₁₀, R₁₂, R₁₃, R₁₄, R₁₅, R₁₇ et R₁₈ sont des groupes alkyle contenant 1 à 12 atomes de carbone; n₁ est égal à 1 -12 et n₂ est égal à 1 15; où R₁, R₂, R₄, R₅, R₆, R₇, R₉ et R₁₀ sont des groupes alkyle contenant 1 à 12 atomes de carbone; R₃ et R₈ sont choisis parmi les groupes alkyle contenant 1 à 12 atomes de carbone, ainsi que l'atome d'hydrogène, n₁ est égal à 1 - 12 et n₂ est égal à 1 - 15; ou R₁, R₂, R₃ et R₄ sont des groupes alkyle contenant 1 à 12 atomes de carbone, n est égal à 1 - 15 et (C₂₆H₅₂N₄)ₙ ou n est égal à 1 - 15.

9. Procédé selon la revendication 8, caractérisé en ce que la composition photochrome contient un ou plusieurs colorants photochromes d'une spiro-oxazine de formule: dans laquelle un des radicaux R₁, R₂ et R₃ est choisi parmi le groupe comprenant un atome d'hydrogène, un atome d'halogène, un groupe alcoxy contenant 1 à 13 atomes de carbone et un groupe alkyle contenant 1 à 12 atomes de carbone, tandis que les autres représentent chacun un atome d'hydrogène; R₄ et R₅ sont choisis parmi le groupe comprenant un atome d'hydrogène, un groupe alkyle contenant 1 à 12 atomes de carbone, un groupe alcoxy contenant 1 à 12 atomes de carbone, un atome d'halogène et un groupe trifluorométhyle, tandis que R₆ représente un groupe alkyle contenant 1 à 12 atomes de carbone.

10. Procédé selon la revendication 9, caractérisé en ce que le stabilisant vis-à-vis de la lumière à base d'une amine à empêchement stérique est choisi parmi un ou plusieurs des composés suivants: le bis-(2,2,6,6-tétraméthyl-4-pipéridinyl)sébaçate; le bis-(1,2,2,6,6-pentaméthyl-4-pipéridinyl)sébaçate; le di-(1,2,2,6,6-pentaméthyl-4-pipéridinyl)-butyl-(3',5'-di-tert.-butyl-4-hydroxybenzyl)malonate; le poly-[(6-[(1,1,3,3-tétraméthylbutyl)-amino]-1,3,5-triazine-2,4-diyl)-(1,6-[2,2,6,6-tétraméthyl-4-pipéridinyl]-amino-hexaméthylène)]; le poly-[[6-(morpholino)-s-triazine-2,4-diyl]-[1,6-(2,2,6,6,-tétraméthyl-4-pipéridyl)-amino]-hexaméthylène]; et le polymère de succinate de diméthyle avec le 4-hydroxy-2,2,6,6-tétraméthyl-1-pipéridine-éthanol.

11. Composition photochrome à base d'une spiro-oxazine dans laquelle est incorporée un stabilisant vis-à-vis de la lumière à base d'une amine à empêchement stérique.

12. Composition photochrome selon la revendication 11, comprenant au moins un composé photochrome répondant à la formule structurale dans laquelle un des radicaux R₁, R₂ et R₃ est choisi parmi le groupe comprenant un atome d'hydrogène, un atome d'halogène, un groupe alcoxy contenant 1 à 12 atomes de carbone, et un groupe alkyle contenant 1 à 12 atomes de carbone, tandis que les autres représentent chacun un atome d'hydrogène; R₄ et R₅ sont choisis parmi le groupe comprenant un atome d'hydrogène, un groupe alkyle contenant 1 à 12 atomes de carbone, un groupe alcoxy contenant 1 à 12 atomes de carbone, un atome d'halogène et un groupe trifluorométhyle, tandis que R₆ représente un groupe alkyle contenant 1 à 12 atomes de carbone; et un stabilisant vis-à-vis de la lumière à base d'une amine à empêchement stérique.

13. Composition selon la revendication 11 comprenant, en outre, un stabilisant extincteur d'oxygène singulet contre l'ultraviolet.

14. Composition selon la revendication 13, caractérisée en ce que ce stabilisant extincteur d'oxygène singulet contre l'ultraviolet est un complexe d'ions Ni²+ avec un coordinat organique.

15. Composition selon la revendication 13, caractérisée en ce que ce stabilisant extincteur d'oxygène singulet contre l'ultraviolet est choisi parmi le [2,2'-thiobis-[4-(1,1,3,3-tétramethylbutyl)phénolato]-(butylamine)]nickel, le [0-éthyl-(3,5-di-tert.-butyl-4-hydroxybenzyl)]phosphonate de nickel, le dibutyldithiocarbamate de nickel, le di-isopropyl-dithiophosphate de nickel, le bis-[2,2'-thiobis-4-(1,1,3,3-tétraméthylbutyl)-phénolato]nickel, le tris-di-n-butyldithiocarbamate de cobalt(III) et le diisopropyldithiocarbamate de cobalt(II).

16. Composition selon une des revendications 11 à 15, caractérisée en ce que le stabilisant vis-à-vis de la lumière à base d'une amine à empêchement stérique est choisi parmi un ou plusieurs composés répondant aux formules suivantes: dans lesquelles R₁, R₂, R₄, R₅, R₆, R₇, R₉ et R₁₀ représentent chacun un groupe alkyle contenant 1 à 12 atomes de carbone, R₃ et R₈ sont choisis parmi un groupe alkyle contenant 1 à 12 atomes de carbone, ainsi qu'un atome d'hydrogène, et n est égal à 1 - 12; où R₁, R₂, R₄, R₅, R₆, R₇, R₉, R₁₀, R₁₁, R₁₂, R₁₃, R₁₄, R₁₅, R₁₆ et R₁₇ représentent chacun un groupe alkyle contenant 1 à 12 atomes de carbone, tandis que R₃ et R₈ sont choisis parmi un groupe alkyle contenant 1 à 12 atomes de carbone, ainsi qu'un atome d'hydrogène; où R₁, R₄, R₅, R₁₁ et R₁₆ sont choisis parmi un groupe alkyle contenant 1 à 12 atomes de carbone, ainsi qu'un atome d'hydrogène, ^{R}2, ^{R}3, ^{R}₇, R₈, ^{R}₉, R₁₀, R₁₂, R₁₃, R₁₄, R₁₅, R₁₇ et R₁₈ représentent chacun un groupe alkyle contenant 1 à 12 atomes de carbone, ni est égal à 1 - 12 et n₂ est égal à 1 - 15; où R₁, R₂, R₄, R₅, R₆, R₇, R₉ et R₁₀ représentent chacun un groupe alkyle contenant 1 à 12 atomes de carbone, R₃ et R₈ sont choisis parmi un groupe alkyle contenant 1 à 12 atomes de carbone, ainsi qu'un atome d'hydrogène, n₁ est égal à 1 -12 et n₂ est égal à 1 - 15; où R₁, R₂, R₃ et R₄ représentent chacun un groupe alkyle contenant 1 à 12 atomes de carbone, et n est égal à 1 - 15; ainsi que (C₂₆H₅₂N₄)ₙ où n est égal à 1 - 15.

17. Composition selon la revendication 16, dans laquelle le stabilisant vis-à-vis de la lumière à base d'une amine à empêchement stérique est choisi parmi un ou plusieurs des composés suivants: le bis-(2,2,6,6-tétraméthyl-4-pipéridinyl)-sébaçate; le bis-(1,2,2,6,6-pentaméthyl-4-pipéridinyl)-sébaçate; le di-(1,2,2,6,6-pentaméthyl-4-pipéridinyl)-butyl-(3',5'-ditert.-butyl-4-hydroxybenzyl)-malonate; le poly-[(6-[(1,1,3,3-tétraméthylbutyl)-amino]-1,3,5-triazine-2,4-diyl)-(1,6-[2,2,6,6-tétraméthyl-4-pipéridinyl]aminohexaméthylène)]; le poly-[[6-(morpholino)-s-triazine-2,4-diyl]-[1,6-(2,2,6,6-tétraméthyl-4-pipéridyl)amino]-hexaméthylène]; et le polymère de succinate de diméthyle avec le 4-hydroxy-2,2,6,6-tétraméthyl-1-pipéridine-éthanol.

18. Composition selon la revendication 16, comprenant, en outre, un hôte plastique.

19. Composition selon la revendication 18 contenant environ 0,1 à environ 15 % en poids du composé photochrome et environ 0,01 à environ 5 % en poids de ce ou de ces stabilisants.

## Revendications (Revendications pour l'(les) Etat(s) contractant(s) suivant(s) : AT)

1. Procédé en vue d'accroître la résistance à la fatigue à la lumière d'une composition photochrome de spiro- oxazine, caractérisé en ce qu'il consiste à incorporer, dans cette composition un stabilisant vis-à-vis de la lumière à base d'une amine à empêchement stérique.

2. Procédé selon la revendication 1, caractérisé en ce Que la composition photochrome contient, en outre, un stabilisant extincteur d'oxygène singulet contre l'ultraviolet.

3. Procédé selon la revendication 2, caractérisé en ce que le stabilisant extincteur d'oxygène singulet contre l'ultraviolet est un complexe d'ions Ni²⁺ avec un coordinat organique.

4. Procédé selon la revendication 2, caractérisé en ce que le stabilisant extincteur d'oxygène singulet contre l'ultraviolet est choisi parmi le [2,2'-thiobis-[4-(1,1,3,3-tétraméthylbutyl)-phénolato]-(butylamine)]-nickel, le [0- éthyl-(3,5-di-tert.-butyl-4-hydroxybenzyl)]-phosphonate de nickel, le dibutyldithiocarbamate de nickel, le di- isopropyl-dithiophosphate de nickel, le bis-[2,2'-thiobis-4-(1,1,3,3-tétraméthylbutyl)-phénolato]-nickel, le tris-di-n-butyldithiocarbamate de cobalt(III) et le diisopropyldithiocarbamate de cobalt(II).

5. Procédé selon une des revendications 1 à 4, caractérisé en ce que la composition photochrome comprend un polymère contenant environ 0,1 à environ 15 % en poids d'un colorant photochrome d'une spiro-oxazine.

6. Procédé selon la revendication 5, caractérisé en ce que le stabilisant vis-à-vis de la lumière à base d'une amine à empêchement stérique et le stabilisant extincteur d'oxygène singulet contre l'ultraviolet sont incorporés dans la composition photochrome en une quantité totale d'environ 0,01 à environ 5 % en poids.

7. Procédé selon la revendication 6, caractérisé en ce que le stabilisant vis-à-vis de la lumière à base d'une amine à empêchement stérique est un dérivé de la tétraméthylpipéridine.

8. Procédé selon une des revendications 1 à 6, caractérisé en ce que le stabilisant vis-à-vis de la lumière à base d'une amine à empêchement stérique est choisi parmi un ou plusieurs composés répondant aux formules suivantes: dans lesquelles R₁, R₂, R₄, R₅, R₆, R₇ R₉ et R₁₀ représentent chacun un groupe alkyle contenant 1 à 12 atomes de carbone, R₃ et R₈ sont choisis parmi un groupe alkyle contenant 1 à 12 atomes de carbone, ainsi qu'un atome d'hydrogène, et n est égal à 1 - 12; où R₁, R₂, R₄, R₅, R₆, R₇, Rg, R₁₀, R₁₁, R₁₂, R₁₃, R₁₄, R₁₅, R₁₆ et R₁₇ représentent chacun un groupe alkyle contenant 1 à 12 atomes de carbone, tandis que R₃ et R₈ sont choisis parmi un groupe alkyle contenant 1 à 12 atomes de carbone, ainsi qu'un atome d'hydrogène; où R₁, R₄, R₅, R₁₁ et R₁₆ sont choisis parmi un groupe alkyle contenant 1 à 12 atomes de carbone, ainsi qu'un atome d'hydrogène, R₂, R₃, R₇, R₈, R₉, R₁₀, R₁₂, R₁₃, R₁₄, R₁₅, R₁₇ et R₁₈ représentent chacun un groupe alkyle contenant 1 à 12 atomes de carbone, n₁ est égal à 1 -12 et n₂ est égal à 1 15; où Rₜ, R₂, R₄, R₅, R₆, R₇, R₉ et R₁₀ représentent chacun un groupe alkyle contenant 1 à 12 atomes de carbone, R₃ et R₈ sont choisis parmi un groupe alkyle contenant 1 à 12 atomes de carbone, ainsi qu'un atome d'hydrogène, nₜ est égal à 1 - 12 et n₂ est égal à 1 - 15; où R₁, R₂, R₃ et R₄ représentent chacun un groupe alkyle contenant 1 à 12 atomes de carbone, tandis que n est égal à 1-15.

9. Procédé selon la revendication 8, caractérisé en ce que la composition photochrome contient plusieurs colorants photochromes de spirooxazine de formule: dans laquelle un des radicaux R₁, R₂ et R₃ est choisi parmi le groupe comprenant un atome d'hydrogène, un atome d'halogène, un groupe alcoxy contenant 1 à 13 atomes de carbone et un groupe alkyle contenant 1 à 12 atomes de carbone, tandis que les autres représentent chacun un atome d'hydrogène; R₄ et R₅ sont choisis parmi le groupe comprenant un atome d'hydrogène, un groupe alkyle contenant 1 à 12 atomes de carbone, un groupe alcoxy contenant 1 à 12 atomes de carbone, un atome d'halogène et un groupe trifluorométhyle, tandis que R₆ représente un groupe alkyle contenant 1 à 12 atomes de carbone.

10. Procédé selon la revendication 9, caractérisé en ce que le stabilisant vis-à-vis de la lumière à base d'une amine à empêchement stérique est choisi parmi un ou plusieurs des composés suivants: le bis-(2,2,6,6-tétraméthyl-4-pipéridinyl)-sébaçate; le bis-(1,2,2,6,6-pentaméthyl-4-pipéridinyl)-sébaçate; le di-(1,2,2,6,6-pentaméthyl-4-pipéridinyl)-butyl-(3',5'-di-tert.-butyl-4-hydroxybenzyl)-malonate; le poly-[(6-[(1,1,3,3-tétraméthylbutyl)-amino]-1,3,5-triazine-2,4-diyl)-(1,6-[2,2,6,6-tétraméthyl-4-pipéridinyl]-amino-hexaméthylène)]; le poly-[[-6-(morpholino)-s-triazine-2,4-diyl]-[1,6-(2,2,6,6-tétraméthyl-4-pipéridyl)amino]-hexaméthylène]; et le polymère de succinate de diméthyle avec le 4-hydroxy-2,2,6,6-tétraméthyl-1-pipéridine-éthanol.

11. Procédé selon la revendication 8 comprenant, en outre, un hôte plastique.

12. Procédé selon la revendication 11, contenant environ 0,1 à environ 15 % en poids du composé photochrome et environ 0,01 à environ 5 % en poids de ce ou de ces stabilisants.
